

## UNITED STATES PATENT OFFICE

2,594,286

## GREASE AND GREASE BASE

William C. Bryant, Garfield, N. J., and Harold Frost, Jr., Yonkers, N. Y., assignors to Swan-Finch Oil Corporation, New York, N. Y., a corporation of New York

No Drawing. Application July 8, 1948,  
Serial No. 37,534

16 Claims. (Cl. 252—51.5)

1

This invention relates to a lubricating composition and particularly to a new type of grease; it also relates to compounds which may be used for producing such grease.

The usual commercial greases heretofore known have consisted of a semi-solid or solid combination of a petroleum product and a soap, or a mixture of soaps, with or without fillers. They have been made by various manufacturing techniques and the soap or soaps serve to produce gelation of the mixture. The usual greases are made up of calcium or soda, or calcium and soda soaps in petroleum oil or other petroleum substances. These known greases have certain disadvantages among which are the following: The lime soap grease and the soda soap grease have poor operating qualities at low temperatures, each producing very high starting torques at low temperatures; for example, at  $-20^{\circ}$  F. Again, when the calcium greases are heated up to the melting point, the water of gelatin boiled off; and when cooled, the soap tends to separate from the oil. When the sodium greases are heated up and cooled, they tend to set to a much heavier mass which is unstable to shearing forces. The calcium greases, furthermore, have relatively low dropping points. Calcium and sodium greases have little rust preventive action and the water-resistance of the sodium greases is quite low. Thus, in contact with water, such greases tend to emulsify and wash away, thus losing their effectiveness.

The principal object of the present invention is to produce a grease which shall overcome at least some of these disadvantages and which shall have superior characteristics to those found in the calcium and sodium greases. Another object of the invention is to provide a suitable base for producing such greases.

The invention comprises the novel products, the specific embodiments of which are described hereinafter by way of example and in accordance with which we now prefer to practice the invention.

We have found in accordance with our invention that a composition containing a proportion of a substance having the formula:



where R is an aliphatic hydrocarbon radical having a carbon chain with a length of C8 to C18, R<sub>1</sub> is an aliphatic hydrocarbon radical having a carbon chain of C2 to C18, and x equals 1 to 8,

2

and in which at least one of said CH<sub>2</sub> groups may be C=CH<sub>2</sub>, mixed with a proportion of a petroleum substance such as various petroleum oils, petrolatum or like substances, possesses useful grease-like characteristics. These greases are in the form of gels and when the compound mentioned above is present in the proportion of about 6 to 18% of the grease, it forms a smooth, semi-solid mass at room temperature. The compound may be used in other proportions, say, from 1 to 35% of the composition, for varying purposes. With 1% composition using a fluid petroleum oil such as cylinder oil, the composition is smooth, thickened with respect to the oil, but is still a fluid.

The amides of the above formula are prepared by amidating corresponding polybasic acids with long chain primary amines. Instead of using a primary amine for such amidation at each end 10 of the chain, we may use at one end of the chain a secondary amine and substances prepared in accordance with such procedure having the formula:



in which R and R<sub>1</sub> are aliphatic hydrocarbon radicals having carbon chains of a length of C8 to C18, and x is as defined above. Substances 30 represented by these formulae are included in our invention. One of the CH<sub>2</sub> groups in Formula A may be substituted by the group, C=CH<sub>2</sub>, in which case the formula then reads:



Examples of the amides employing long chain 40 primary and secondary amines and their characteristics, useful for making compositions or grease bases in accordance with our invention are given below. All of the following compounds have been prepared by us. All of them are opaque, amorphous solids varying in color from white to light amber. All of them are soluble in petroleum oils and other organic solvents and are substantially insoluble in water. The odor of these substances varies from ammoniacal for 45 those containing short aliphatic chains such as the N-lauryl-N<sub>1</sub>-n-butyl-sebacamide to sweet-spicy for those containing all long chains attached to the nitrogen atoms. Each of these substances may be produced by the same process, 50 for which a typical process example follows:

## 3

## Process example

For making N-stearyl-N<sub>1</sub>-oleyl-sebacamide,

203 gms. of sebacic acid were melted and 216 gms. of stearylamine were added thereto slowly. The mass was held at a temperature to assure the half salt being liquid at all times. After all of the stearylamine had been added, all of the oleylamine (214 gms.) was added at the same time, and the temperature raised to 300° F. and maintained at 300° F. for three hours.

## Yield, per cent

|             |       |
|-------------|-------|
| Theoretical | 95.13 |
| Actual      | 95.09 |

The material obtained is an amorphous solid with a slightly spicy odor. It is light amber in color.

The amide is an unsymmetrical amide and the different amines are added separately as above indicated in making this amide and the others listed below. In making the symmetrical amides listed below, the total quantity of the single amine used may be added all at once.

The yield so obtained in the above example represents the compound recovered after all the water of reaction has been removed. In the description of each of the substances given below, the yield obtained is given and was obtained in the same manner as that described in the above example.

The above example employs a temperature of 300° F. for the reaction. For the manufacture of the other below-listed amides correspondingly produced by the above example, the temperature will vary in a range of 250° F. to 350° F. As the chain length of the acid used increases, the temperature employed must be raised correspondingly, but all temperatures employed will be within the range stated.

Each of the capillary melting points given below are sharp melting points. In the case of the compounds designated "Tech.," corresponding to the compounds mentioned below, the capillary melting points will have a short range. In these technical materials also, the actual range will start at a somewhat lower point, about 3° C., below the capillary melting point of the relatively pure material. Also, in these technical compounds, the nitrogen content will be slightly higher, namely, up to about 0.1% nitrogen.

The said examples of the amides employing long chain primary and secondary amines and their characteristics are as follows:

N-lauryl-N<sub>1</sub>-lauryl-azelaamide

|             | Analysis         |                   |                   | Yield             |
|-------------|------------------|-------------------|-------------------|-------------------|
|             | Nitrogen         | Hydrogen          | Carbon            |                   |
| Theoretical | Per cent<br>5.37 | Per cent<br>12.65 | Per cent<br>75.90 | Per cent<br>93.56 |
| Actual      | 5.15             | 12.71             | 75.87             | 93.18             |

The product is an opaque, amorphous solid having a cream color. It has a spicy odor. Its melting point is 104° C. capillary; 229° F. American wax melting point. In preparing this amide, the lauryl amine was combined with the azelaic

75

above example for the process.

## 4

acid and amidated for three hours at 300° F. in accordance with the above example for the process.



|        | Analysis         |                   |                   | Yield             |
|--------|------------------|-------------------|-------------------|-------------------|
|        | Nitrogen         | Hydrogen          | Carbon            |                   |
| 15     | Per cent<br>4.32 | Per cent<br>12.96 | Per cent<br>77.72 | Per cent<br>94.74 |
| Actual | 4.29             | 12.91             | 77.80             | 94.68             |

The product is an opaque, amorphous solid having a light cream color. It has a spicy odor.

20 Its melting point is 114° C. capillary; 238° F. American wax melting point. In preparing this amide, the palmityl amine was combined with the sebacic acid and amidated for three hours at 300° F. in accordance with the above example for the process.

N-lauryl-N<sub>1</sub>-oleyl azelaamide

|        | Analysis         |                   |                   | Yield             |
|--------|------------------|-------------------|-------------------|-------------------|
|        | Nitrogen         | Hydrogen          | Carbon            |                   |
| 30     | Per cent<br>4.28 | Per cent<br>12.91 | Per cent<br>77.80 | Per cent<br>94.68 |
| Actual | 4.29             | 12.91             | 77.80             | 94.68             |

## Yield, per cent

|             |       |
|-------------|-------|
| Theoretical | 94.28 |
| Actual      | 94.20 |

35 The product is an opaque, amorphous solid having a light amber color. It has a slightly spicy odor. Its melting point is 101° C. capillary; 217° F. American wax melting point. In preparing this amide, the lauryl amine and oleyl amine were combined with the azelaic acid and amidated for three hours in accordance with the above example for the process.

N-stearyl-N<sub>1</sub>-stearyl-itaconamide

|        | Analysis         |                   |                   | Yield             |
|--------|------------------|-------------------|-------------------|-------------------|
|        | Nitrogen         | Hydrogen          | Carbon            |                   |
| 45     | Per cent<br>5.37 | Per cent<br>12.65 | Per cent<br>75.90 | Per cent<br>93.56 |
| Actual | 5.15             | 12.71             | 75.87             | 93.18             |

## Yield, per cent

|             |       |
|-------------|-------|
| Theoretical | 93.94 |
| Actual      | 93.90 |

50 The product is an opaque, white amorphous solid. It has a spicy odor. Its melting point is 118° C. capillary; 241° F. American wax melting point. In preparing this amide, the stearyl amine was combined with the itaconic acid and amidated in accordance with the above example for the process, employing a temperature of 260° F. for one hour.

N-lauryl-N<sub>1</sub>-n-butyl-sebacamide

|        | Analysis         |                   |                   | Yield             |
|--------|------------------|-------------------|-------------------|-------------------|
|        | Nitrogen         | Hydrogen          | Carbon            |                   |
| 60     | Per cent<br>5.37 | Per cent<br>12.65 | Per cent<br>75.90 | Per cent<br>93.56 |
| Actual | 5.15             | 12.71             | 75.87             | 93.18             |

## Yield, per cent

|             |       |
|-------------|-------|
| Theoretical | 92.16 |
| Actual      | 92.11 |

65 The product is an opaque, amorphous solid having a light cream color. It has a slightly ammoniacal odor. Its melting point is 114° C. capillary; 239° F. American wax melting point. In preparing this amide, the lauryl and n-butyl amine were combined with the sebacic acid and amidated for three hours in accordance with the above example for the process.



be used in a mixture of amines having approximately the following composition:

|                  | Per cent | Per cent |
|------------------|----------|----------|
| Primary amines   |          | 85       |
| Octyl amine      | 8        |          |
| Decylamine       | 9        |          |
| Dodecylamine     | 47       |          |
| Tetradecylamine  | 18       |          |
| Hexadecylamine   | 8        |          |
| Octadecylamine   | 5        |          |
| Octadecenylamine | 5        |          |
| Secondary amines |          | 15       |
| Total            |          | 100      |

This mixed amine would, of course, produce a mixture of corresponding amides with the dibasic acid selected.

Examples of amides employing secondary amines in accordance with the formula



where  $\text{R}$ ,  $\text{R}_1$  and  $x$  are as defined above, are as follows:



Yield, per cent

|             |       |
|-------------|-------|
| Theoretical | 96.04 |
| Actual      | 96.01 |

The product is an opaque, white, amorphous solid with a slightly spicy odor. In preparing this amide, the lauryl and stearyl amines were combined with the sebacic acid and amidated in accordance with the above example for the process.



Yield, per cent

|             |       |
|-------------|-------|
| Theoretical | 96.09 |
| Actual      | 96.04 |

The product is an opaque, light amber, amorphous solid with a slightly spicy odor. In preparing this amide, the oleyl and palmityl amines were combined with the azelaic acid and amidated in accordance with the above example for the process.



Yield, per cent

|             |       |
|-------------|-------|
| Theoretical | 95.77 |
| Actual      | 95.70 |

The product is an opaque, cream colored, amorphous solid with a slightly spicy odor. In preparing this amide, the lauryl and palmityl amines were combined with the sebacic acid and amidated in accordance with the above example for the process.



Yield, per cent

|             |       |
|-------------|-------|
| Theoretical | 96.14 |
| Actual      | 96.11 |

The product is an opaque, light amber, amorphous solid with a slightly spicy odor. In preparing this amide, the oleyl and palmityl amines were combined with the sebacic acid and amidated in accordance with the above example for the process.

The reaction which occurs for the production of the material in accordance with Formula A above is as follows:

10 (1)



15 where  $\text{R}$ ,  $\text{R}_1$  and  $x$  are as defined above. Of course, if  $\text{R}$  and  $\text{R}_1$  represent the same radical, the equation can be simplified to recite

(2)



If a secondary amine is used, the reaction is represented as follows:

25



30  $\text{R}$  may be  $\text{R}_1$  in this reaction. In other words,  $\text{R}$  and  $\text{R}_1$  are used herein to indicate radicals of dissimilar chain length.

The following are examples of the manner in which we now prefer to practice our invention for the manufacture of grease. These examples are illustrative and the invention is not to be considered as confined thereto except as indicated in the appended claims.

#### Example 1

|                                                                   | Per cent |
|-------------------------------------------------------------------|----------|
| N-lauryl-N <sub>1</sub> -lauryl-sebacamide                        | 10       |
| 100/100° F. S. S. U. (Seconds Saybolt Universal) Coastal pale oil | 90       |
|                                                                   | 100      |

45 The amide and the oil are heated together to 275° F. to effect solution, and the molten mass is allowed to cool to room temperature with constant slow (40 R. P. M.) agitation until the mass forms a smooth, semi-solid mass.

50 The semi-solid mass is allowed to cool to room temperature (70-85° F.) and the mass is agitated slowly until the mass has a smooth, clear appearance and the penetration is stable according to ASTM D-217-47 T (Amer. Soc. for Testing Materials Specification D-217-47). The resultant grease had the following characteristics:

|                                                                        |               |
|------------------------------------------------------------------------|---------------|
| Penetration 5000 strokes working                                       | 380           |
| Penetration ASTM D-217-47-T                                            | 335           |
| D/P (drop point) ASTM D-566/42                                         | 215° F.       |
| D/P Chrysler 461-C-31                                                  | 206° F.       |
| 65 BEC (Bearing Engineers Committee machine) starting torque at 70° F. | 420 dynes     |
| BEC running torque at 70° F.                                           | 240 dynes     |
| BEC starting torque at -20° F.                                         | 1260 dynes    |
| 70 BEC running torque at -20° F.                                       | 300 dynes     |
| Corrosion test—greases—F. S. B. 791b                                   | Nil           |
| Rust protection 10% salt spray                                         | 72 hrs. O. K. |
| Water absorption (Chrysler 461-C-41)                                   | 20%           |

For purposes of comparison, we give below corresponding characteristics, respectively, of lime and soda soap greases:

A lime soap grease, 10% soap, 90% 100/100° F. S. S. U. Coastal pale oil had the following characteristics:

Penetration 5000 strokes working ----- 420  
 Penetration ASTM D-217-47-T ----- 330  
 D/P ASTM D-566-42 ----- 188° F.  
 D/P Chrysler 461-C-31 ----- 181° F.  
 BEC starting torque at 70° F. ----- 540 dynes  
 BEC running torque at 70° F. ----- 120 dynes  
 BEC starting torque at -20° F. ----- Over 2700 dynes  
 BEC running torque at -20° F. ----- No stable point  
 (continued to drop)

Corrosion test—grease—F. S. B. 791b (Federal Specification Book VVL) ----- Nil  
 Rust protection 10% salt spray 8 hrs. failed  
 Water absorption Chrysler 461-C-41 ----- 10%

A sodium soap grease, 10% soda soap, 90% 100/100° F. S. S. U. Coastal pale oil had the following characteristics after being milled smooth:

Penetration 5000 strokes working ----- Over 420  
 Penetration ASTM D-217-47-T ----- 342  
 D/P ASTM D-566-42 ----- 300° F.  
 D/P Chrysler 461-C-31 ----- 240° F.  
 BEC starting torque at 70° F. ----- 540 dynes  
 BEC running torque at 70° F. ----- 180 dynes  
 BEC starting torque at -20° F. ----- Over 2700 dynes  
 BEC running torque at -20° F. ----- 600 dynes  
 Corrosion test—grease—F. S. B. 791b ----- Nil  
 Rust protection 10% salt spray 10 hrs. failed  
 Water absorption Chrysler 461-C-41 ----- At 60% turned to liquid emulsion

The above characteristics show that the amide grease is superior to the calcium grease in all respects and is superior to the sodium grease in many respects. With respect to the sodium grease, it is noted that there is very little syneresis in the amide grease as compared with the sodium grease, as may be seen by comparing the dropping points of the two. The difference between ASTM D-566-42 dropping point and the Chrysler 461-C-41 dropping point is interpreted as being indicative of bleeding (syneresis) tendency of a grease. The greater the numerical difference of the two dropping points, the greater the bleeding tendency. As can be seen from the data above, the difference on the invention product listed is only nine (9) whereas for the sodium grease example the difference is sixty (60). Furthermore, the amide grease has a sharp melting point and does not thin out over a wide temperature range. The amide greases when compounded as above revert to their original gel structure after being heated to the melting point and allowed to cool, whereas the calcium greases show separation of the soap from the oil upon cooling and the sodium greases set to a much heavier mass that is unstable to shearing action when so heated and cooled.

#### Example 2

Per cent  
 N-tech. lauryl-Ni-tech. lauryl-sebacamide ----- 6  
 2000/100° F. S. S. U. mineral oil blend (Mid-Continent) ----- 94

The amide and the oil were heated together to 270° F. to achieve complete solution. The mixture was allowed to cool to room temperature over night. The solid mass was milled out to a smooth, buttery consistency. The following characteristics appeared on test:

Penetration ASTM D-217-47-T ----- 340  
 D/P ASTM D-566-42 ----- °F. 226

10 The other properties of this grease were similar to those given under Example 1.

#### Example 3

|                                             | Per cent |
|---------------------------------------------|----------|
| N-tech. lauryl-Ni-tech. lauryl-sebacamide   | 6        |
| 15 3500/100° F. S. S. U. residual black oil | 94       |
|                                             | 100      |

The same compounding technique was followed as in Example 2. The following characteristics appeared on test:

Penetration ASTM D-217-47-T ----- 330  
 D/P ASTM D-566-42 ----- °F. 222

25 The other properties of this grease were similar to those given under Example 1.

#### Example 4

|                                           | Per cent |
|-------------------------------------------|----------|
| N-tech. lauryl-Ni-tech. lauryl-sebacamide | 4        |
| 30 98% 200-mesh graphite                  | 14       |
| 3500/100° F. S. S. U. residual black oil  | 82       |
|                                           | 100      |

The amide and the oil were heated together to 270° F. to effect solution, and the mass slowly stirred while cooling until the mass formed a heavy plastic mass. The graphite was stirred in slowly to prevent lumping. After the graphite was all in, and the batch was smooth, the mass was allowed to cool to room temperature. When cool, the mass was milled to a smooth, unctuous lubricating grease. The following characteristics appeared on test:

45 Penetration ASTM D-217-47-T ----- 310  
 D/P ASTM D-566-42 ----- °F. 222

The other properties of this grease were similar to those given under Example 1.

#### Example 5

|                                           | Per cent |
|-------------------------------------------|----------|
| N-tech. lauryl-Ni-tech. lauryl-sebacamide | 15       |
| 50 70/100° F. pale paraffin oil           | 85       |
|                                           | 100      |

55 The same compounding technique was followed as in Example 1. The following characteristics appeared on test:

Penetration ASTM D-217-47-T ----- 275  
 60 D/P ASTM D-566-42 ----- °F. 230

The other properties of this grease were similar to those given under Example 1.

#### Example 6

|                                           | Per cent |
|-------------------------------------------|----------|
| N-tech. lauryl-Ni-tech. lauryl-sebacamide | 12       |
| 65 300/100° F. white oil                  | 88       |
|                                           | 100      |

70 The same compounding technique was followed as in Example 2. The following characteristics appeared on test:

Penetration ASTM D-217-47-T ----- 290  
 75 D/P ASTM D-566-42 ----- °F. 231

## 11

The other properties of this grease were similar to those given under Example 1.

## Example 7

|                                                        | Per cent |
|--------------------------------------------------------|----------|
| N-tech. lauryl-N <sub>1</sub> -tech. lauryl-azelaamide | 10       |
| 100/100° F. S. S. U. Coastal pale oil                  | 90       |
|                                                        | 100      |

The same compounding technique was followed as in Example 1. The following characteristics appeared on test:

|                             |        |
|-----------------------------|--------|
| Penetration ASTM D-217-47-T | 345    |
| D/P ASTM D-566-42           | °F 205 |

The other properties of this grease were similar to those given under Example 1.

## Example 8

|                                                                   | Per cent |
|-------------------------------------------------------------------|----------|
| N-tech. lauryl-N <sub>1</sub> -tech. oleyl-azelaamide             | 10       |
| 160/100° F. S. S. U. solvent extracted Mid-<br>continent pale oil | 90       |
|                                                                   | 100      |

The same compounding technique was followed as in Example 1. The following characteristics appeared on test:

|                             |        |
|-----------------------------|--------|
| Penetration ASTM D-217-47-T | 325    |
| D/P ASTM D-566-42           | °F 200 |

The other properties of this grease were similar to those given under Example 1.

## Example 9

|                                               | Per cent |
|-----------------------------------------------|----------|
| N-stearyl-N <sub>1</sub> -stearyl-itaconamide | 10       |
| 300/100° F. S. S. U. Coastal pale oil         | 90       |

100

The same compounding technique was followed as in Example 1. The following characteristics appeared on test:

|                             |        |
|-----------------------------|--------|
| Penetration ASTM D-217-47-T | 350    |
| D/P ASTM D-566-42           | °F 203 |

The other properties of this grease were similar to those given under Example 1.

## Example 10

|                                                  | Per cent |
|--------------------------------------------------|----------|
| N-lauryl-N <sub>1</sub> -mono-n-butyl-sebacamide | 10       |
| 100/100° F. S. S. U. Coastal pale oil            | 90       |

100

The same compounding technique was followed as in Example 1. The following characteristics appeared on test:

|                             |        |
|-----------------------------|--------|
| Penetration ASTM D-217-47-T | 275    |
| D/P ASTM D-566-42           | °F 265 |

The other properties of this grease were similar to those given under Example 1.

## Example 11

|                                                        | Per cent |
|--------------------------------------------------------|----------|
| N-tech. lauryl-N <sub>1</sub> -tech. lauryl sebacamide | 1        |
| 4000/100° F. S. S. U. Coastal bright stock             | 99       |

100

The same compounding technique was followed as in Example 1. Formed a solution that was a true gel but was of a semi-fluid consistency. Using a 30 gm. cone, in place of the 150 gm.

## 12

cone, the following characteristics appeared on test:

|                                    |        |
|------------------------------------|--------|
| Penetration Modified ASTM D-217-47 | 330    |
| D/P ASTM D-566-42                  | °F 135 |

The other properties of this grease were similar to those given under Example 1.

## Example 12

|                                                        | Per cent |
|--------------------------------------------------------|----------|
| N-tech. lauryl-N <sub>1</sub> -tech. lauryl sebacamide | 2        |
| 500/100° F. S. S. U. Coastal pale oil                  | 98       |
|                                                        | 100      |

The same compounding technique was followed as in Example 1. Formed a true gel of semi-solid character. With a 30 gm. cone, the following characteristics appeared on test:

|                           |        |
|---------------------------|--------|
| Penetration ASTM D-217-47 | 300    |
| D/P ASTM D-566-42         | °F 155 |

The other properties of this grease were similar to those given under Example 1.

## Example 13

|                                                       | Per cent |
|-------------------------------------------------------|----------|
| N-tech lauryl-N <sub>1</sub> -tech. lauryl sebacamide | 20       |
| 100/100° F. S. S. U. Coastal pale oil                 | 80       |
|                                                       | 100      |

The same compounding technique was followed as in Example 1. The following characteristics appeared on test:

|                           |        |
|---------------------------|--------|
| Penetration ASTM D-217-47 | 275    |
| D/P ASTM D-566-42         | °F 245 |

The other properties of this grease were similar to those given in Example 1.

## Example 14

|                                                        | Per cent |
|--------------------------------------------------------|----------|
| N-tech. lauryl-N <sub>1</sub> -tech. lauryl sebacamide | 35       |
| 100/100° F. S. S. U. Coastal pale oil                  | 65       |

The same compounding technique was followed as in Example 1. The following characteristics appeared on test:

|                           |        |
|---------------------------|--------|
| Penetration ASTM D-217-47 | 205    |
| D/P ASTM D-566-42         | °F 265 |

The other properties of this grease were similar to those given in Example 1.

## Example 15

|                                              | Per cent |
|----------------------------------------------|----------|
| N-lauryl-N <sub>1</sub> -palmityl malonamide | 10       |
| 500/100° F. S. S. U. Coastal pale oil        | 90       |

The same compounding technique was followed as in Example 2. The following characteristics appeared on test:

|                           |        |
|---------------------------|--------|
| Penetration ASTM D-217-47 | 355    |
| D/P ASTM D-566-42         | °F 190 |

The other properties of this grease were similar to those given in Example 1.

Although we prefer the compounds made with primary amines, we have also produced useful

## 13

compounds employing the secondary amines, as follows:

## Example 16

Per cent

|                                                  |     |
|--------------------------------------------------|-----|
| N-lauryl-N <sub>1</sub> -sec. stearyl-sebacamide | 10  |
| 300/100° F. S. S. U. Coastal pale oil            | 90  |
|                                                  | 100 |

This grease was made in the same manner as in Example 1. The following characteristics appeared on test:

|                             |         |
|-----------------------------|---------|
| Penetration ASTM D-217-47-T | 340     |
| D/P ASTM D-566-42           | °F. 211 |

The other properties of this grease were similar to those given in Example 1.

## Example 17

Per cent

|                                                   |     |
|---------------------------------------------------|-----|
| N-lauryl-N <sub>1</sub> -sec. palmityl-sebacamide | 10  |
| 300/100° F. S. S. U. Coastal pale oil             | 90  |
|                                                   | 100 |

This grease was made in the same manner as in Example 1. The following characteristics appeared on test:

|                             |         |
|-----------------------------|---------|
| Penetration ASTM D-217-47-T | 310     |
| D/P ASTM D-566-42           | °F. 210 |

The other properties of this grease were similar to those given in Example 1.

## Example 18

Per cent

|                                                  |     |
|--------------------------------------------------|-----|
| N-oleyl-N <sub>1</sub> -sec. palmityl sebacamide | 10  |
| 300/100° F. S. S. U. Coastal pale oil            | 90  |
|                                                  | 100 |

This grease was made in the same manner as in Example 1. The following characteristics appeared on test:

|                             |         |
|-----------------------------|---------|
| Penetration ASTM D-217-47-T | 306     |
| D/P ASTM D-566-42           | °F. 209 |

The other properties of this grease were similar to those given in Example 1.

The greases made in accordance with our invention, as pointed out, are non-metallic products. They are homogeneous; that is, the organic gelling agent is compatible in all respects with the petroleum oil or similar substance, causing the product to act as a chemical entity. Accordingly, the greases do not separate on storage or when subjected to high heat under operating conditions. In other words, they do not "bleed" under such conditions. They possess in general increased film strength. They show increased shear resistance, demonstrated by the fact that upon rupture of the film, it tends to heal itself quickly. They have increased oxidation stability. They give rust protection to the metal being lubricated. This has been verified by salt spray tests. In addition, they show better water-repellency. They also possess reversibility, namely, the grease will melt and then on cooling will revert to its gel form. They have a wide temperature range of operation. Tests both at low and high temperatures have demonstrated this. Due to the fact that the grease bases contain at least one hydrogen atom attached to one or more of the nitrogen groups, these bases are polar which will cause the lubricant, even in melted condition, to adhere to the metal being lubricated. In addition, tests have shown that the greases possess greater oiliness.

## 14

Subject matter described but not claimed herein is claimed in copending application Serial No. 220,124, filed April 3, 1951.

What we claim is:

1. A grease composition comprising a petroleum lubricant and a sufficient quantity of a gelation agent to cause at least a partial gelation thereof, said agent being selected from the group consisting of



in which R and R<sub>1</sub> are aliphatic hydrocarbon radicals, R having a carbon chain of a length of C8 to C18, R<sub>1</sub> having a carbon chain of a length of C2 to C18, and x equals 1 to 8.

2. A grease composition comprising a petroleum lubricant and a sufficient quantity of a gelation agent to cause at least a partial gelation thereof, said agent having the formula



where R and R<sub>1</sub> are aliphatic hydrocarbon radicals, R having a carbon chain of a length of C8 to C18, R<sub>1</sub> having a carbon chain of a length of C2 to C18, and x equals 1 to 8.

3. A grease composition comprising a major proportion of a petroleum lubricant and a minor proportion of a gelation agent, said agent having a formula



where R and R<sub>1</sub> are aliphatic hydrocarbon radicals, R having a carbon chain of a length of C8 to C18, R<sub>1</sub> having a carbon chain of a length of C2 to C18, and x equals 1 to 8.

4. A grease having a grease base in the proportion of 1 to 35% of the total weight of the grease having the formula



where R and R<sub>1</sub> are aliphatic hydrocarbon radicals, R having a carbon chain of a length of C8 to C18, R<sub>1</sub> having a carbon chain of a length of C2 to C18, and x equals 1 to 8, and the major proportion of the remainder of the grease being composed of petroleum oil.

5. A grease having about 6 to 18% of grease base having the formula



where R and R<sub>1</sub> are aliphatic hydrocarbon radicals, R having a carbon chain of a length of C8 to C18, R<sub>1</sub> having a carbon chain of a length of C2 to C18, and x equals 1 to 8, and the remainder being composed substantially of petroleum oil.

6. A grease having up to 14% graphite and about 4% technical N-lauryl-N<sub>1</sub>-lauryl-sebacamide, the remainder of the grease being composed substantially of mineral oil.

7. A grease composed of about 10% of N-tech. lauryl-N<sub>1</sub>-tech. lauryl-azelaamide and the remainder being composed substantially of mineral oil.

8. A grease composed of about 10% of N-tech. lauryl-N<sub>1</sub>-tech. oleyl-azelaamide and the remain-

15

der being composed substantially of mineral oil.

9. A grease composed of about 10% of N-stearyl-N<sub>1</sub>-stearyl-itaconamide and the remainder being composed substantially of mineral oil.

10. A grease composed of about 10% of N-<sup>5</sup>tech. lauryl-N<sub>1</sub> mono n butyl-sebacamide and the remainder being composed substantially of mineral oil.

11. As a new composition, a mixture containing a minor proportion of a substance having the <sup>10</sup> formula



where R and R<sub>1</sub> are aliphatic hydrocarbon radicals, R having a carbon chain of a length of C<sub>8</sub> to C<sub>18</sub>, R<sub>1</sub> having a carbon chain of a length of C<sub>2</sub> to C<sub>18</sub>, the balance of the composition being a petroleum lubricant.

12. A process in accordance with claim 2 in which the gelation agent is N-lauryl-N<sub>1</sub>-lauryl-<sup>20</sup> azelaamide.

13. A process in accordance with claim 2 in which the gelation agent is N-lauryl-N<sub>1</sub>-oleyl-<sup>25</sup> azelaamide.

14. A process in accordance with claim 2 in

16

which the gelation agent is N-lauryl-N<sub>1</sub>n-butyl-sebacamide.

15. A process in accordance with claim 2 in which the gelation agent is N-lauryl-N<sub>1</sub>-lauryl-<sup>5</sup> sebacamide.

16. A process in accordance with claim 2 in which the gelation agent is N-stearyl-N<sub>1</sub>-stearyl-itaconamide.

WILLIAM C. BRYANT.  
HAROLD FROST, JR.

## REFERENCES CITED

The following references are of record in the file of this patent:

## UNITED STATES PATENTS

| Number    | Name           | Date          |
|-----------|----------------|---------------|
| 1,659,149 | Nill           | Feb. 14, 1928 |
| 1,937,463 | Nill           | Nov. 28, 1933 |
| 2,109,941 | D'Alelio       | Mar. 1, 1938  |
| 2,304,475 | Pool           | Dec. 8, 1942  |
| 2,364,737 | McGrew         | Dec. 12, 1944 |
| 2,371,104 | Kienle et al.  | Mar. 6, 1945  |
| 2,412,708 | Blair          | Dec. 17, 1946 |
| 2,417,833 | Lincoln et al. | Mar. 25, 1947 |
| 2,490,744 | Trigg et al.   | Dec. 6, 1949  |